

July 31, 1934.

B. LIEBOWITZ

1,968,410

APPAREL

Filed May 31, 1933



INVENTOR.  
Benjamin Liebowitz  
BY *Leventhal & Liebowitz*

ATTORNEY.

## UNITED STATES PATENT OFFICE

1,968,410

## APPAREL

Benjamin Liebowitz, New York, N. Y., assignor to  
Trubenizing Process Corporation, New York,  
N. Y., a corporation of New York

Application May 31, 1933, Serial No. 673,695

12 Claims. (Cl. 2—131)

This invention relates to apparel, and constitutes an improvement of patent application Serial Number 603,242, filed by me on April 5th, 1932.

In the following specification I shall describe my invention with particular reference to the manufacture of collars, including collar bands, both of the attached and detached types. It is to be clearly understood, however, that the invention is not limited to collars but applies as well to the manufacture of cuffs, parts of shirts, or other articles of apparel formed of a plurality of plies or pieces of textile fabric.

An object of the invention is to provide commercially practical means for cementing or binding together, either in whole or in part, the plies or pieces of a collar or other article of apparel.

Another object is to provide cementing means, the use of which does not in any way interfere with the usual methods of manufacturing the article.

A further object is to provide a process whereby the cementing of the plies or pieces, or such portions thereof as it may be desired to cement together, is effected after the article has been in essentials completely manufactured.

Other objects are to provide a collar or like article which is permeable to water and air so that it may be readily laundered and is comfortable to wear; which is in whole or in part stiffened to a desired degree without the use of starch or any extraneous stiffening means; and, which will withstand repeated laundering without substantially losing its initial stiffness.

A collar made according to this invention is similar in outward appearance to an ordinary soft or semi-stiff collar of the same style but is more durable, lasting in shape, and resistant to wilting from perspiration or heat, rumpling in wear, or wrinkling in washing and ironing than the ordinary collar. Compared with a starched collar, it has suitable body without being too stiff, and is far more comfortable to wear.

In the practice of the invention, as will be hereinafter more fully explained, I cement the parts or plies together by means of a lining fabric composed in part or entirely of yarns of a substance, such as a suitable cellulose derivative, which is non-cementitious in itself but which is capable of being made cementitious by subsequent treatment.

I am aware that it has been proposed in the prior art to bind together and stiffen portions of the plies of a collar or like article by coating or impregnating the fabric with a cementitious

solution of cellulose in a solvent. This method waterproofs the article and makes it impermeable both to moisture and air, and, therefore, a coated collar is uncomfortable to wear in warm weather as it does not allow perspiration of the neck to pass through. Such a collar is also difficult to launder properly for while the surfaces may be washed, the body of the collar cannot be thoroughly cleaned because water will not penetrate it in the ordinary laundering operation. Furthermore, it is apparent that the application of a cementitious solution, because of its adhesive nature, entails considerable difficulty and inconvenience in handling the treated parts and fabricating the collars. Collars of that character cannot be made by usual turning method generally employed in collar factories but have to be made by a special method wherein the edges are untreated with the adhesive and are subsequently turned in as a separate operation to simulate the appearance of the customary turned edges. Also, in the case of a folding collar, the adhesive binding material is omitted along the region of the fold or hinge.

The accompanying drawing illustrates an embodiment of the invention applied to a folded collar of the attached type, in which:—

Figure 1 is a view of the collar laid flat and unfolded, with a portion of the fabric broken away to show the lining;

Figure 2 is a diagrammatic plan view of a piece of the lining, greatly magnified;

Fig. 3 is a view corresponding to Fig. 2 and showing the lining applied to the collar band, portions of the band being broken away to disclose the lining and the inner ply; and

Fig. 4 is an enlarged section showing the collar folded.

Referring now to the drawing, the lining material, one example of which is illustrated on a magnified scale in Fig. 2, consists of a woven fabric composed of yarns or threads 1 of cotton or other suitable substance, and additional yarns or threads 2 of a suitable cellulose derivative of such character as to be capable of being made cementitious by treatment with a suitable solvent.

The yarns 2 may be made of any suitable cellulose derivative, such as a cellulose ester, as, for example, cellulose acetate, or of a suitable cellulose ether, as, for example, ethyl cellulose. In making the yarns 2, the particular cellulose derivative selected may be used alone, or in connection with suitable plasticizers, or other substances, not necessarily plasticizers, which will

60

65

70

75

80

85

90

95

100

105

110

have a beneficial effect on the cellulose derivative, as, for instance, increasing its resistance to the alkaline detergents used in laundering.

While, preferably, the lining is made of both cotton and cellulose derivative yarns, it is to be understood that it may be made entirely of yarns of cellulose derivative substance. Furthermore, while in the particular example illustrated I have shown the cellulose derivative yarn used only in the warp, it may be used both in the warp and the filler, or in the filler alone.

In certain cases, as, for example, where it is desired to bind and stiffen only certain portions of the collar, such as the wings, points, or along the edges, the use of the cellulose derivative in the lining may be confined to those portions, and in such cases, if desired, ordinary lining material may be used in the other portions of the collar.

In making the collar, the lining 3, and the two fabric pieces or plies 4 and 5 are cut or blanked out as usual, and are both laid on one side of the lining, and united along three edges by a line of stitching 6. The assemblage is then turned in the manner usual in the art to form turned-in edges and to bring the lining 3 on the inside in position between the two fabric plies 4 and 5. The points of the collar are then pressed and the parts are again sewed together by the usual line of stitching 7, after which the band 8 is attached in the usual manner by the customary stitching 9.

When the collar has in essentials been completely fabricated, it is treated with acetone, ethyl acetone, or any other suitable solvent for the particular cellulose derivative used, which has the property of rendering the cellulose derivative yarns 2 of the lining adhesive but which will not affect the cotton yarns 1 or the outer fabric plies of the collar. The solvent is applied from the outside and is allowed to soak into the lining through the outer fabric plies 4 and 5. A convenient way of applying the solvent is to place the collar between two pads that are kept moistened or saturated with the solvent. Treatment with the solvent is continued for a sufficient length of time to moisten the cellulose derivative substance sufficiently to make it cementitious or adhesive. Heat and pressure are then applied to the collar so as to bind the outer plies to the lining and to stiffen the collar. It will be understood that the collar may be stiffened and cemented either before or after it is attached to the collar band 8.

In order that the collar shall be permeable to water and air, the weave of the lining is preferably so constructed, with respect to the diameter and spatial relation of the yarns, that when the cellulose derivative yarns are treated with the solvent, the substance of said yarns will not film over and fill the interstices of the weave.

Usually the special lining material 3 is confined to the collar proper, the band 8 being lined with ordinary lining material. However, if desired, the special lining material 3 may be used both in the collar proper and the band. Figs. 3 and 4 show a construction wherein the lining material 3 is applied both to the collar and to the band. The band is of conventional construction comprising outer and inner fabric plies 10 and 11, which plies are attached to the edge portion 12 of the collar proper, below the fold 13, by the usual concealed stitches 14, as well as the exposed stitches 9. The lower edge of the band shown in these views is left free for attachment to the shirt, but it will be understood that in making a collar of the detached type, said lower edge may be finished as usual. It will also be noted that the lining 3 of the collar

proper extends over the fold line 13, which may be conveniently determined by folding the collar after the stitching operations are completed and subjecting it to heat and pressure to make a firm crease along the fold line.

The special lining material 3 that I use for cementing and stiffening the plies of the collar may be handled in the manner of the ordinary linings commonly used and does not in any way interfere with carrying out the usual method of making the collar or other article of apparel.

A collar made according to this invention may be of any desired degree of stiffness but I prefer usually to make it of the stiffness commonly known in the art as "semi-stiff", that is, stiffer than the ordinary soft collar but not as stiff as a fully starched collar.

The method of cementing herein described, involving a binding agent which is used initially in a non-cementitious state but which is made cementitious by subsequent treatment, does not discolor or otherwise affect the appearance of the material of the cemented plies or parts. This is important, particularly in connection with the manufacture of colored shirts and collars, because to produce a commercially satisfactory product it is necessary that the shirt and collar, whether the latter be of the attached or detached type, match exactly in shade and color. On the other hand, the use of a liquid or plastic cementing substance applied to the plies or to the lining, as has heretofore been proposed, tends to discolor the material and to produce spots or blotches when the plies are pressed together.

According to the provisions of the patent statutes, I have described the principle and characteristics of my invention together with the preferred manner of practicing it and several variations and modifications thereof. However, I desire to have it understood that, within the scope of the appended claims, the invention may be practiced otherwise than specifically described herein.

What I claim is:—

1. A moisture pervious article of apparel of the character described, made of fabric plies cemented together by a fabric having woven therein a substance which is initially non-cementitious but has the inherent property of being made cementitious.

2. An article of apparel of the character described, made of fabric plies cemented together by a woven fabric comprising cellulose derivative yarn of such character as to become cementitious upon treatment with a suitable solvent.

3. An article of apparel of the character described, made of fabric plies cemented together by a woven fabric comprising cellulose ester yarn of such character as to become cementitious upon treatment with a suitable solvent.

4. An article of apparel of the character described, made of fabric plies cemented together by a woven fabric comprising cellulose ester yarns of such character as to become cementitious upon treatment with acetone.

5. A moisture and air permeable stiffened collar or like article made of inner and outer fabric plies, and an intermediate woven lining comprising in its construction yarn of a cellulose derivative substance of such character as to become cementitious by treatment with a solvent, said inner and outer fabric plies being cemented to the lining by the adhesion of the cellulose derivative substance of the lining.

6. A moisture pervious semi-stiff collar having

80

85

90

95

110

115

120

125

130

135

140

145

150

outer and inner fabric plies cemented to an intermediate lining fabric having woven therein a substance which is initially non-cementitious, but which is capable of being made cementitious, after the collar is in essentials completely fabricated so as to bind said outer and inner plies to the lining.

7. A moisture pervious semi-stiff collar having outer and inner fabric plies cemented to an intermediate lining fabric, said lining fabric having woven therein a substance which is inherently capable of being made cementitious.

8. The process of cementing fabric parts of an article of apparel which comprises disposing between the parts to be cemented a piece of fabric woven with yarn made of a cellulose derivative substance, applying to said parts, from the outside, a solvent which will penetrate through the fabric and make the cellulose derivative substance cementitious, and applying pressure to bind the parts together.

9. The process of cementing fabric parts of an

article of apparel which comprises disposing between the parts to be cemented a piece of fabric woven with yarn made of a cellulose ester, applying acetone to said parts, from the outside, so that the acetone will penetrate through the fabric and make the cellulose ester cementitious, and applying heat and pressure to bind the parts together.

10. A moisture pervious article of wearing apparel comprising plies of fabric stiffened and adhesively secured together by an intermediate layer of textile lining material having cellulose derivative threads interwoven therewith.

11. A moisture pervious article of apparel comprising a plurality of plies of fabric one or more of which has adhesive material interwoven therewith.

12. A moisture pervious article of apparel comprising a plurality of plies of fabric adhesively secured together by means of adhesive material interwoven with one or more of said plies.

80

85

90

95

100

1,968,410.—*Benjamin Liebowitz, New York, N. Y. APPAREL. Patent dated July 31, 1934. Disclaimer filed May 17, 1939, by the assignee, Celanese Corporation of America.*

Hereby enters this disclaimer to claims 1, 6, 7, 8, and 10 of said specification.  
[Official Gazette June 13, 1939.]

105

35

110

40

115

45

120

50

125

55

130

60

135

65

140

70

145

75

150

outer and inner fabric plies cemented to an intermediate lining fabric having woven therein a substance which is initially non-cementitious, but which is capable of being made cementitious, after the collar is in essentials completely fabricated so as to bind said outer and inner plies to the lining.

7. A moisture pervious semi-stiff collar having outer and inner fabric plies cemented to an intermediate lining fabric, said lining fabric having woven therein a substance which is inherently capable of being made cementitious.

8. The process of cementing fabric parts of an article of apparel which comprises disposing between the parts to be cemented a piece of fabric woven with yarn made of a cellulose derivative substance, applying to said parts, from the outside, a solvent which will penetrate through the fabric and make the cellulose derivative substance cementitious, and applying pressure to bind the parts together.

9. The process of cementing fabric parts of an

article of apparel which comprises disposing between the parts to be cemented a piece of fabric woven with yarn made of a cellulose ester, applying acetone to said parts, from the outside, so that the acetone will penetrate through the fabric and make the cellulose ester cementitious, and applying heat and pressure to bind the parts together.

10. A moisture pervious article of wearing apparel comprising plies of fabric stiffened and adhesively secured together by an intermediate layer of textile lining material having cellulose derivative threads interwoven therewith.

11. A moisture pervious article of apparel comprising a plurality of plies of fabric one or more of which has adhesive material interwoven therewith.

12. A moisture pervious article of apparel comprising a plurality of plies of fabric adhesively secured together by means of adhesive material interwoven with one or more of said plies.

80

85

90

95

100

1,968,410.—*Benjamin Liebowitz, New York, N. Y.* APPAREL. Patent dated July 31, 1934. Disclaimer filed May 17, 1939, by the assignee, *Celanese Corporation of America*.

Hereby enters this disclaimer to claims 1, 6, 7, 8, and 10 of said specification.  
[Official Gazette June 13, 1939.]

105

35

110

40

115

45

120

50

125

55

130

60

135

65

140

70

145

75

150